

## UNITED STATES PATENT OFFICE

2,082,840

## PROCESSES OF PRODUCING YARN

James Louis Lohrke, Thornbury Township,  
Delaware County, Pa.No Drawing. Application April 13, 1935,  
Serial No. 16,158

5 Claims. (Cl. 18—1)

The present invention relates to a process of producing yarn from so-called endless or continuous textile fibers and to the yarn so produced, and is an improvement on the invention of Patent No. 1,883,384, issued to me and Henry H. Perry on October 18, 1932.

In the invention of our said patent we produce a yarn from a continuous sliver composed of a multiplicity of substantially continuous fibers grouped in substantial parallelism, by reducing the fibers to staple fibers while maintaining their substantial parallelism and the continuity of the sliver, by simultaneously or thereafter drafting the resulting sliver, and by then suitably 15 twisting such resulting sliver to produce a yarn or a roving from which the yarn is subsequently formed.

In our said patent, we disclose a specific embodiment of the invention in which the reducing 20 step, above referred to, is performed in and by the drafting of the sliver. This is an important feature of the patented invention, since we discovered that by making a continuous sliver composed of a multiplicity of substantially continuous 25 conventional fibers grouped in substantial parallelism and drafting such a sliver, the continuous fibers could be reduced to staple fibers. We also discovered that in thus reducing the continuous fibers to staple fibers, they were 30 broken in a haphazard manner into irregular staple lengths, and that the substantial parallelism of the fibers would be maintained. We further discovered that such haphazard breaking 35 would produce a proper imbrication of the staple fibers so that the continuity of the sliver would also be maintained.

In the simultaneous breaking and drafting of the sliver of substantially continuous fibers the length of the staple fibers produced is determined, within limits, by adjusting the drafting mechanism. For instance, where sets of drafting rollers are employed, the length of the staple fibers desired in the yarn is determined by what is known as setting the ratch, which is the distance 45 between the sets of drafting rollers. The drafting mechanism is adjusted or set for the maximum length of staple fibers to be produced in the breaking operation. In this way the length of the staple fibers is varied, in the practice of our 50 patented process, to suit the character of yarn to be produced thereby and the steps and/or machinery thereafter employed in such production.

In so practicing the process of our Patent No. 1,883,384, however, difficulty is experienced when 55 endeavoring to break the substantially continuous fibers to relatively short staple lengths, such, for example, as are suitable for spinning on conventional machinery according to the cotton system, because of the fact that the setting of the 60 ratch for such relatively short staple lengths is

interfered with by the relatively large drafting rollers which are preferably used in carrying out the simultaneous breaking and drafting operation in order to apply sufficient pressure to the sliver to prevent slippage of the fibers without crushing or otherwise damaging the same.

It has also been found in practicing the invention of our patent, that in the production of relatively short staple lengths for finer counts of 5 yarn such as made by the cotton system, the fibers composing the sliver sometimes break in bunches instead of in a haphazard manner, so that there is a lack of proper imbrication, and a tendency of the sliver to draft unevenly and perhaps break down or lose its continuity.

By the present invention I overcome these difficulties, and according to it the sliver of substantially continuous or endless fibers is first tensioned, as by drafting rollers, to break the fibers to produce over-size staple lengths, that is, 10 staple lengths substantially greater than desired for the yarn, and the resulting sliver is thereafter subjected to one or more tensioning operations, as by drafting rollers, to reduce the over-size 15 staple lengths so that the same are not greater than, and as far as possible are substantially 20 equal to, the staple length desired for the production of the finished yarn, the continuity of the 25 sliver and the parallelism of the fibers being maintained throughout the successive operations.

The preferred manner of practicing the present 30 invention is as follows:—

There is first made an endless or continuous sliver composed of a multiplicity of substantially 35 endless or continuous fibers brought together or combined in substantial parallelism. This sliver is passed through two sets of drafting rollers, that is, sets of feed and of delivery rollers, in 40 which the rollers of the respective sets travel at the same surface speed but the surface speed of the delivery rollers is greater than that of the feed rollers. Each set may consist of any suitable number of rollers. The ratch of such sets of drafting rollers is suitably adjusted so as 45 to be substantially longer than the length of staple desired in the yarn to be produced. As the sliver passes through these sets of drafting rollers, tension is applied to successive portions 50 of the fibers which are of a length corresponding to the setting of the ratch, and as a result of this tension the fibers are broken to over-size staple lengths, that is, to staple lengths substantially greater than, and preferably approximately twice, that desired for the yarn. This breaking 55 occurs in a haphazard manner, producing irregular staple lengths, a large portion of which are over-size although some staple lengths less than over-size may be produced owing to the haphazard breaking. The relative speeds of the 60

feed and delivery rollers are preferably such that the staple fibers produced are subjected to a simultaneous drafting operation which attenuates and suitably reduces the size of the sliver. The

5 haphazard breaking produces a proper imbrication of the staple fibers so that the continuity of the sliver is maintained. Furthermore, the substantial parallelism of the fibers in the resulting sliver is preserved.

10 Thereafter, the resulting sliver is passed through the feed and delivery rollers of another tensioning and drafting mechanism in which the ratch is adjusted so as to be substantially equal to the length of staple desired for the yarn to be produced. In this operation the over-size 15 staple fibers are broken so that they are less than but as far as possible substantially equal to the staple length desired for the yarn. This breaking occurs in a haphazard manner as in the previous operation and hence some of the 20 staple fibers may be shorter than the desired staple length. The simultaneous drafting further reduces the size of the resulting sliver. The continuity of the resulting sliver and the substantial 25 parallelism of the fibers thereof, are both maintained as in the previous operation.

Following the second breaking and drafting operation, the resulting sliver is twisted in any well-known or suitable manner, as, for instance, 30 according to the cotton system, to produce a relatively short staple, fine count yarn directly therefrom.

In carrying out the present invention in this 35 preferred manner it has been found that excellent results are obtained by setting the ratch of the first breaking and drafting mechanism at about 7 1/4 inches, and by setting the ratch of the second breaking and drafting mechanism at about 40 3 1/2 inches. These specific settings are given, however, merely by way of example, and are not to be construed as a limitation upon the invention.

It has also been found that when the substantially continuous fibers composing the sliver 45 have been broken to staple fibers of over-size lengths in the first operation, the breaking in the second operation can be performed satisfactorily by drafting rollers of a size which will 50 not interfere with the setting of the ratch necessary to produce the relatively short staple fibers desired for the yarn.

An important advantage of the present invention 55 is that the yarn produced by this improved process is more even, that is, of more uniform size, than relatively short staple yarn produced by the process of Patent No. 1,883,384, and has substantially greater tensile strength.

While the improved process has been described 60 in connection with a single sliver of substantially endless fibers, it will be understood that two or more slivers of staple fibers produced by the breaking operations heretofore described may be combined if desired. For example, two of the 65 slivers resulting from the first breaking operation may be combined and the subsequent breaking operation carried out upon the sliver thus formed.

It will also be understood that the practice of 70 the invention is not limited to the employment of two breaking operations as disclosed in connection with the preferred method herein described, but it may be carried out in more than two operations so long as the endless fibers are first broken

to over-size staple lengths and the over-size staple lengths are subsequently broken to staple lengths not greater than the staple length desired in the yarn.

What I claim is:

1. In the process of producing yarn from a sliver composed of a multiplicity of substantially continuous fibers grouped in substantial parallelism, while maintaining the substantial parallelism of the fibers and the continuity of the sliver, applying tension to successive portions of said fibers to progressively break the fibers to over-size staple length, and thereafter applying tension to the over-size staple lengths thus produced to break the same to staple fibers having a 15 length not greater than that desired in the yarn.

2. In the process of producing yarn from a sliver composed of a multiplicity of substantially continuous fibers grouped in substantial parallelism, while maintaining the substantial parallelism of the fibers and the continuity of the sliver, applying tension to successive portions of the fibers, having a length substantially greater than the maximum length of the staple desired in the yarn, to progressively break the fibers in 25 a haphazard manner, and thereafter applying tension to the over-size staple fibers thus produced to break the same to staple lengths not greater than desired in the yarn, and drafting the resulting sliver.

3. In the process of producing yarn from a sliver composed of a multiplicity of substantially continuous fibers grouped in substantial parallelism, while maintaining the substantial parallelism of the fibers and the continuity of the sliver, applying tension to successive portions of said fibers to progressively break the same to over-size staple lengths and simultaneously draft the sliver, and thereafter applying tension to such over-size staple lengths to break the same 40 to staple fibers of not greater than the length desired in the yarn and to simultaneously draft the resulting sliver.

4. The process of producing yarn which consists in making a continuous sliver composed of a multiplicity of substantially continuous fibers grouped in substantial parallelism, passing the sliver through a group of drafting rollers having a ratch substantially greater than the maximum length of staple desired in the yarn to thereby 50 break the fibers to staple fibers some of which are over-size and to draft the sliver, and thereafter passing the resulting sliver through a second group of drafting rollers having a ratch substantially equal to the length of the staple desired in the yarn thereby to break the over-size 55 staple fibers and to draft the sliver, while maintaining the substantial parallelism of the fibers and the continuity of the sliver.

5. In the process of producing yarn from a continuous sliver composed of a multiplicity of substantially continuous conventional fibers grouped in substantial parallelism, reducing the fibers to staple fibers and drafting the sliver while maintaining both the substantial parallelism of the fibers and the continuity of the sliver, by passing the sliver through a plurality of groups of drafting rollers, the initial group having a ratch substantially greater than the maximum length of staple desired in the yarn and the final group 70 having a ratchet substantially equal to such maximum length.

JAMES LOUIS LOHRKE.